

## 1

3,129,100

DEVELOPING ACCELERATORS FOR SILVER  
HALIDE EMULSION LAYERS

Herbert Grabhöfer, Cologne-Flittard, Horst Schüler, Munich, and Hans Ulrich and August Randolph, Leverkusen, Germany, assignors to Agfa Aktiengesellschaft, Leverkusen, Germany, a corporation of Germany

No Drawing. Filed Mar. 13, 1962, Ser. No. 179,472  
Claims priority, application Germany Mar. 16, 1961  
6 Claims. (Cl. 96—66)

This invention concerns a new class of developing accelerators which are chemically characterized by at least one quaternary nitrogen atom substituted by a cyanoethoxyethyl radical as well as a process for developing silver halide emulsion layers.

It has long been known that quaternary nitrogen compounds are able to accelerate photographic development, whether as an additive to the developer or to the emulsion. It was originally assumed that the effect depends on the action of the cation on surface tension, such as can be produced for example by longer aliphatic radicals. As shown by subsequent investigations this limitation is not necessary (see for example *Angewandte Chem.*, vol. 67, page 523 (1955)).

All onium salts are similar in their action to the quaternary nitrogen compounds, for example quaternary phosphonium or ternary sulphonium salts. One or more charged onium groups may be present in the molecule.

It is also known that this action of the onium compounds is obtained with systems which are sensitized with polyalkylene oxides; the emulsions used can also be spectrally sensitized. Moreover, intramolecular linkages of polyalkylene oxides with quaternary ammonium salts have been briefly described.

The effect of the acceleration of the development which has been referred to can be explained according to T. H. James, *Photographic Science and Technique*, vol. 19B (1953), page 35, by the fact that the negatively charged bromine ion shell which exists around the silver halide grain is neutralized by the onium cations thus facilitating access of the negatively charged developer anions for example the hydroquinone anion with a double negative charge in an alkaline medium which is normally made difficult because of electrostatic repulsion of said ion shell. The higher the charge on the developer anion, the greater is the shortening of the latent period by the addition of suitable quaternary salts.

In conformity with this theory, onium salts are most highly effective as development accelerators when alkali developers containing solely hydroquinone as developer compound are used.

Some of the known onium salts still show a good accelerating effect with the super additive metol-hydroquinone development system which is of importance in practice, but scarcely any effects with strongly super additive systems such as 1-phenyl-3-pyrazolidone/hydroquinone or p-aminophenyl-3-aminopyrazoline/hydroquinone. With the last-mentioned system, in which for example the 1-p-aminophenyl-3-aminopyrazoline enters into a reciprocal action with the silver halide grain and thus constitutes the reaction which determines the speed of development, a further increase in the speed of development was not to be expected on account of the already very short latent periods per se (see *Phot. Science and Engin.*, vol. 4, page 225 (1960)).

It is among the objects of the instant invention to provide compounds which further accelerate the development and shorten the latent period even with strongly super additive developer systems.

It has now been found that considerable acceleration

## 2

effects can still be produced if the development is carried out in the presence of quaternary nitrogen compounds of the general formula:



in which  $\text{R}_1$  and  $\text{R}_2$  stand for alkyl, aralkyl, phenyl, cyanoethyl, or cyanoethoxyethyl or for methylene groups or 10 atoms necessary for completing a heterocyclic ring such as morpholine, piperidine and the like;  $\text{R}_3$  represents alkyl, aralkyl, phenyl, cyanoethoxyethyl or a radical selected from those having the following general formulae



and



wherein  $\text{R}_1$  and  $\text{R}_2$  have the meaning specified above;  $\text{X}$  represents any desired anion, such as a halide, toluene-sulfonate or alkyl sulphate anion. It may be pointed out that the anion is not especially critical and is selected according to the requirements of the special composition or emulsion in which the compound is to be used;  $m$  is an integer from 2-5,  $n$  from 2-6 and  $p$  from 1-100, preferably 1-7.

30 The ethylene oxide chains of the compounds represented by the above general formula can be replaced with other alkylene oxide chain such as propylene oxide or butylene oxide chains.

35 The excellent and surprising efficacy of the compounds according to the invention as well as their superiority over similar known products rests apparently on the action of the cyanoethyl and cyanethyl oxethyl radicals.

The quaternary salts can either be added to the developer or to the emulsion or to both simultaneously.

40 The acceleration effect of the compounds according to the invention is not restricted to certain types of emulsions or developers. It is also apparent with color developers containing aromatic amine developing compounds or with emulsions containing optical or chemical sensitizers such as sulphur compounds, salts of precious metals such as ruthenium, rhodium, palladium, iridium or platinum, furthermore, iodine salts, reducing agents, polyalkylene oxides, mercuric compounds, stabilizing agents such as compounds of the azaindene series, e.g., 4-hydroxy-6-methyl-1,3,3a,7-tetra-azaindene. The accelerators according to the invention can also be advantageously used with fixing developers. They may also surprisingly be used at the same time as anti-fogging agents.

45 55 Examples of the new development accelerators are those of the following constitution:



60 Dimethyl-phenethyl-cyanoethoxyethyl-ammonium chloride



65 Diethyl-benzyl-cyanoethoxyethyl-ammonium chloride



70 Di-(n-butyl)-benzyl-cyanoethoxyethyl-ammonium chloride





The aforementioned quaternary salts may be prepared as follows:

## COMPOUND I

(a) *N,N-Dimethyl-N-Cyanoethoxyethylamine*

2 g. of sodium methylate are dissolved in 89.1 g. (1 mol) of dimethylaminoethanol and 53 g. (1 mol) of stabilized acrylonitrile are added at 35° C. while stirring. After standing for 5 hours at room temperature, 200 cc. of water and 10 cc. of 25 percent sodium hydroxide solution are added and the mixture is shaken three times, using 250 cc. of methylene chloride on each occasion. The methylene chloride phase is separated, dried with sodium sulfate and concentrated by evaporation. The remaining amine is fractionated in vacuum.

B.P. 73-74°/0.9 torr. Yield: 82 g.

(b) *Dimethyl-Phenethyl-Cyanoethoxyethyl-Ammonium Chloride*

14.2 g. of the aforementioned amine (Ia) and 14 g. of 2-chloroethyl benzene are heated while stirring for 2 hours to 150° C., 100 cc. of acetone and the quantity of ethanol (about 10 ml.) necessary for forming a solution are then added. On cooling, 88 g. of quaternary salt with a melting point of 123° C. crystallize out.

## COMPOUND II

(a) *N,N-Diethyl-N-Cyanoethoxyethylamine*

117 g. of diethylaminoethanol and 100 g. of sodium hydroxide are dissolved in 250 cc. of water and 53 g. of acrylonitrile are added dropwise while stirring at 45° C. The mixture is left standing for 5 hours at room temperature and is then extracted by shaking three times with methylene chloride, using 250 cc. on each occasion. After distilling off the methylene chloride, an oil is left which is fractionated in vacuo.

B.P. 134° C./16 torr. Yield: 105 g.

(b) *Diethylbenzyl-Cyanoethoxyethyl-Ammonium Chloride*

12.5 g. of benzyl chloride and 14.6 g. of the aforementioned amine (IIa) are heated for 2 hours while stirring to 150° C. The mixture is stirred with 50 cc. of acetone with heating and cooled with iced water. Crystals with a melting point of 91° C. are obtained.

Yield: 12 g.

## COMPOUND III

(a) *N,N-Dibutyl-N-Cyanoethoxyethylamine*

2 g. of sodium methylate are dissolved in 173 g. of di-n-butylethanolamine and 53 g. of acrylonitrile are added while stirring at 35° C. The mixture is left for 6 hours at room temperature and is then stirred with 200 cc. of water, 10 cc. of 25 percent sodium hydroxide solution and 500 cc. of methylene chloride. 155 g. of amine with the boiling point 169° C./13.5 torr are recovered from the methylene chloride phase after vacuum distillation.

(b) *Di-n-Butyl-Benzyl-Cyanoethoxyethyl-Ammonium Chloride*

12.7 g. of benzyl chloride and 22.6 g. of the aforementioned amine (IIIa) are heated in 50 ml. of dry toluene for 16 hours to boiling point. The crystals precipitating on cooling are suction-filtered and washed with ether.

M.P. 160° C. Yield: 8 g.

## COMPOUND IV

*Dimethyl-(p)-Chlorobenzyl-Cyanoethoxyethyl-Ammonium Bromide*

14.2 g. of N,N-dimethyl-N-cyanoethoxyethylamine (Ia) and 20.5 g. of 4-chlorobenzyl bromide are thoroughly

5

mixed at room temperature. After 1 hour, crystals have separated out, and these are washed with acetone.

M.P. 133° C. Yield: 30 g.

## COMPOUND V

*Dimethyl-4-Nitrobenzyl-Cyanoethoxyethyl-Ammonium Chloride*

14.2 g. of N,N-dimethyl-N-cyanoethoxyethyl (Ia) and 17.1 g. of p-nitrobenzyl chloride are heated for 5 hours under reflux in 50 cc. of acetone. The precipitated crystals are suction-filtered and recrystallized from a mixture of acetone and alcohol (10:1).

M.P. 144-145° C. Yield, 22 g.

## COMPOUND VI

(a) *N-Methyl-N,N-Di(Cyanoethoxyethyl)-Amine*

119 g. of N-methyl-N,N-di-( $\beta$ -hydroxyethyl)-amine and 10 g. of sodium hydroxide are dissolved in 250 cc. of water and 106 g. of acrylonitrile are added thereto at 45° C. within 1 hour. The mixture is left for 8 hours at room temperature. Thereafter, 30 g. of sodium hydroxide are added and the amine precipitated as an oil is taken up in methylene chloride. After distilling off the methylene chloride, the amine is fractionated in vacuo.

B.P. 160-170° C./0.9-1.5 torr. Yield, 55 g.

(b) *Methyl-4-Chlorobenzyl-di(Cyanoethoxyethyl)-Ammonium Bromide*

21.9 g. of the aforementioned amine (VIa) and 20.5 g. of p-chlorobenzyl bromide are heated for 1 hour to 150° C. The mixture is thereafter stirred with 50 cc. of acetone at boiling temperature. The product crystallized out is washed on a suction filter several times with acetone.

M.P. 159° C. Yield: 32.5 g.

40

22.6 g. of N,N-di-n-butyl-N-cyanoethoxyethyl-amine (IIIa) and 14 g. of  $\beta$ -chlorethyl benzene are heated under reflux for 6 hours in 50 cc. of dry toluene. After standing for 15 hours at room temperature, crystals are separated out and these are suction-filtered and washed several times with ether. M.P. 158° C. Yield: 16 g.

## COMPOUND VII

*Di - n - Butyl - Phenethyl - Cyanoethoxyethyl-Ammonium Chloride*

22.6 g. of N,N-di-n-butyl-N-cyanoethoxyethyl-amine (IIIa) and 14 g. of  $\beta$ -chlorethyl benzene are heated under reflux for 6 hours in 50 cc. of dry toluene. After standing for 15 hours at room temperature, the precipitated oil is separated out and treated with acetone. The crystals which are thereby formed are suction-filtered and washed several times with ether.

M.P. 70° C. Yield: 12 g.

60

*Dibutyl - Phenethyl - Cyanoethoxyethyl-Ammonium Chloride*

22.6 g. of N,N-di-(n-butyl)-N-cyanoethoxyethyl amine (IIIa) and 20.5 g. of p-chlorobenzyl bromide are heated for 30 minutes to 150° C. After standing for 8 hours at room temperature, the product is dissolved while hot in acetone and precipitated with ether.

Crystals have a melting point of 80° C. Yield 25 g.

70

## COMPOUND X

*Dimethyl-n-Octyl-Cyanoethoxyethyl-Ammonium Bromide*

14.2 g. of N,N-dimethyl-N-cyanoethoxyethyl-amine (Ia) and 19.3 g. of n-octyl bromide are heated for 2 hours to

75

100° C. The reaction product is recrystallized from acetone.

M.P. 98-99° C. Yield: 21 g.

#### COMPOUND XI

##### *Diethyl-n-Octyl-Cyanoethoxyethyl-Ammonium Bromide*

17 g. of N,N-diethyl-N-cyanoethoxyethyl amine (IIa) and 19.3 g. of n-octyl bromide are heated for 2 hours to 100° C. After standing for 24 hours in a refrigerator, the product is triturated with ether and suction-filtered.

M.P. 55-58° C. Yield: 20 g.

#### COMPOUND XII

##### *Dimethyl-n-Dodecyl-Cyanoethoxyethyl-Ammonium Bromide*

14.2 g. of N,N-dimethyl-N-cyanoethoxyethyl amine (Ia) and 24.9 g. of dodecyl bromide are heated for 2 hours to 100° C. The reaction product is recrystallized from acetone.

M.P. 107° C. Yield: 28 g.

#### COMPOUND XIII

##### *1,6-Hexamethylene-Bis-[N,N,N',N'-Tetramethyl-N,N'-Di-(Cyanoethoxyethyl)]-Ammonium Bromide*

14.2 g. of N,N-dimethyl-N-cyanoethoxyethyl amine (Ia) and 12.2 g. of 1,6-dibromohexane are heated for 2 hours to 100° C. The reaction product is recrystallized from a mixture of acetone and alcohol (10:2).

M.P. 144° C. Yield: 21 g.

#### COMPOUND XIV

##### *1,6-Hexamethylene-Bis-[N,N,N',N'-Tetraethyl-N,N'-Di-(Cyanoethoxyethyl)]-Ammonium Bromide*

17 g. of N,N-diethyl-N-cyanoethoxyethyl amine (IIa) and 12.2 g. of 1,6-dibromohexane are heated for 2 hours to 100° C. After adding 50 cc. of acetone, the mixture is heated for 1 hour under reflux, cooled and suction-filtered. Recrystallization takes place from acetone/alcohol (10:2).

M.P. 151° C. Yield: 12 g.

#### COMPOUND XV

##### *(a) N,N-Di(Cyanoethyl)-N-(Cyanoethoxypropyl)Amine*

75 g. of 3-amino-1-propanol and 10 g. of sodium hydroxide are dissolved in 250 cc. of water and 159 g. of acrylonitrile are added in portions at 45° C. while stirring. After stirring for 8 hours, the mixture is extracted three times by shaking with methylene chloride, using 250 cc. on each occasion. The combined extracts are washed with 50 cc. of water, dried with sodium sulphate, filtered and concentrated by evaporation. The residue is fractionated under vacuum.

B.P. 160° C./0.5 torr. Yield: 120 g.

##### *(b) N,N-Di(Cyanoethyl)-N-4-Chlorobenzyl-N-(Cyanoethoxypropyl)Ammonium Bromide*

4.7 g. of N,N-di(cyanoethyl)-N-(cyanoethoxypropyl) amine (XVa) and 4.1 g. of p-chlorobenzyl bromide are heated for 3 hours to 150° C.; the product is then treated with acetone and precipitated with ether.

M.P. 127° C. Yield: 2.8 g.

#### COMPOUND XVI

##### *Ethylene-Bis-[N,N,N',N'-Tetra-Methyl-N,N'-Di-(Cyanoethoxyethyl)]-Ammonium-Bromide*

Prepared according to Compound XIII using 1,2-dibromoethane as starting compound.

#### COMPOUND XVII

##### *(a) Diethylene-Glycol-Di-Methane-Sulphonic Acid Ester*

114.5 g. of methane-sulfo-chloride are added in portions at 0° C. to a solution of 53 g. of diethylene glycol in 200 cc. of dried pyridine. After stirring for 1 hour

at 10° C. the mixture is poured on ice water, acidified with aqueous hydrochloride, separated with common salt and shaken three times each with 300 cc. of methylene chloride. The collected methylene chloride extracts are dried with sodium sulphate and evaporated. Crystals are obtained having a melting point of 55-56° C. after recrystallization from alcohol.

##### *(b) Ethoxyethyl - $\alpha,\omega$ - Bis - [N,N,N',N' - Tetramethyl-N,N'-Di-(Cyanoethoxyethyl)] - Ammonium - Methane Sulfonate*

26.2 g. of di-ethylene glycol di-methane sulfonic acid ester (XVIIa) and 28.4 g. of  $\beta$ -cyanoethoxyethyl-N-dimethylamine (Ia) are mixed and heated on an oil bath for 4 hours to a temperature of 120° C. The reaction mixture is extracted three times with hot benzene for separating undesired side products, dissolved in methyl alcohol and this solution clarified with active carbon, bleaching earth and again with active carbon. The filtrate is completely evaporated. After heating to 100° C. in vacuo, 39 g. of a yellowish viscous sirupy liquid remain. Yield 71 percent of the theory.

A 20 percent aqueous solution is used for photographic applications.

#### COMPOUND XVIII

##### *(a) Triethylene Glycol Di-p-Toluene Sulfonic Acid Ester*

75 g. of triethylene glycol dissolved in 200 cc. of dried pyridine are reacted with 190 g. of toluene sulpho-chloride at 0° C. Further processing is accomplished according to Example XVII. A crystallized compound is obtained which melts after recrystallization from ethanol at 73-74° C.

##### *(b) Di - (Ethoxy) - Ethyl - $\alpha,\omega$ - Bis - [N,N,N',N' - Tetra-methyl - N,N' - Di - (Cyanoethoxyethyl)] - Ammonium-p-Toluene Sulfonate*

45.2 g. of triethylene glycol di-p-toluene sulphonic acid ester (XVIIia) and 28.4 g. of  $\beta$ -cyanoethoxyethyl-N-dimethylamine (Ia) are heated for 4 hours to a temperature of 120° C. The reaction mixture is further processed as described in Example XVIIc. 50 g. (68 percent of the theory) of a yellow colored sirupy liquid are obtained.

#### COMPOUND XIX

##### *(a) Ethoxyethyl - $\alpha,\omega$ - Bis - [N,N'-Dimethyl-N,N,N',N'-Tetra-(Cyanoethoxyethyl)]Ammonium-Methane Sulfonate*

10.4 g. of diethylene glycol di-methane sulfonic acid ester (XVIIa) and 17.2 g. of di-( $\beta$ -cyanoethoxyethyl)-N-methylamine (VIa) are thoroughly mixed, heated in an oil bath for 4-5 hours at 130° C. and thereafter further processed as described in Example XVIIc. 21 g. (74 percent of the theory) of a yellowish brown sirupy liquid are obtained.

#### COMPOUND XX

##### *Di - (Ethoxy) - Ethyl - $\alpha,\omega$ - Bis - [N,N' - Dimethyl - N, N,N' - Tetra - (Cyanoethoxyethyl)] - Ammonium-Toluene Sulfonate*

45 g. of triethylene glycol di-p-toluene sulfonic acid ester (XVIIia) and 45 g. of di-( $\beta$ -cyanoethoxyethyl)-N-methylamine (VIa) are heated for 5 hours to a temperature of 120° C. and further processed as described in Example XVIIc. 58.5 g. (65 percent of the theory) of a yellowish brown sirupy liquid are obtained.

#### COMPOUND XXI

##### *(a) $\gamma$ -Cyanoethoxypropyl-N,N-Di(Cyanoethyl)-Amine*

159 g. of acrylonitrile are added in portions with stirring at 45° C. to a solution of 75 g. of 3-aminopropanol (1) and 10 g. of sodium hydroxide in 250 cc. of water. After stirring for 8 hours the mixture is shaken three times with 250 cc. of methylene chloride each. The collected extracts are washed with 50 cc. of water, dried

## 11

with sodium sulphate, filtrated and evaporated. The residue is fractionated in vacuo.

B.P. 160° C./0.5 torr.

(b) *Ethoxyethyl- $\alpha,\omega$ -Bis-[N,N,N',N'-Tetracyanethyl-N,N'-Di-(Cyanoethoxypropyl)]-Ammonium-Methane Sulfonate*

47 g. of  $\gamma$ -cyanoethoxypropyl-N,N-dicyanethyl-amine (XXIa) and 26.2 g. of diethylene glycol di-methane sulfonic acid ester (XVIIa) are heated for 4 hours at 120° C. and further processed according to Example XVIIc. 52 g. (71 percent of the theory) of a yellowish brown sirupy liquid are obtained.

## COMPOUND XXII

(a) *Diethyl-Cyanoethoxypropyl-Amine*

53 g. of acrylonitrile are added dropwise with stirring at 45° C. to a solution of 159 g. of diethylamino pentanol-(5) (described in J. Am. Soc. 69 (1947), page 2581) and 10 g. of sodium hydroxide in 250 cc. of water. The mixture is left standing for 10 hours at room temperature and is shaken thereafter three times with 250 cc. of methylene chloride each. The combined extracts are evaporated and the remaining oil fractionated in vacuo.

B.P. 165° C./12 torr.

(b) *Di-(Ethoxy)-Ethyl- $\alpha,\omega$ -Bis-[N,N,N',N'-Tetraethyl-N,N'-Di-(Cyanoethoxypropyl)]-Ammonium-p-Toluene Sulfonate*

42.4 g. of diethyl-cyanoethoxypropyl-amine (XXIIa) and 45.2 g. of triethylene glycol di-p-toluene sulfonic acid ester (XVIIa) are heated for 5 hours to 120° C. Further processing is accomplished as described in Example XVIIc. 55 g. (63 percent of the theory) of a yellowish brown sirupy liquid are obtained which solidifies on supercooling to the waxy product.

## COMPOUND XXIII

*Di-(Ethoxy)-Ethyl- $\alpha,\omega$ -Bis-N,N'-[Hexa-(Cyanoethoxyethyl)]-Ammonium-p-Toluene Sulfonate*

61.6 g. of tri-(cyanoethoxyethyl)-amine (described in United States Patent No. 2,326,721) and 45.2 g. of triethylene glycol di-p-toluene sulfonic acid ester (XVIIa) are heated for 5 hours to 120° C. and further processed according to Example XVIIc. 80 g. (75 percent of the theory) of a high viscous product are obtained.

## COMPOUND XXIV

*Di-(Ethoxy)-Ethyl- $\alpha,\omega$ -Bis-[N,N'-Diethyl-N,N'-Diphenyl-N,N'-Di-(Cyanoethoxyethyl)]-Ammonium-p-Toluene Sulfonate*

46.4 g. of  $\beta$ -cyanoethoxyethyl-N-phenyl-N-ethyl amine (described in United States Patent No. 2,326,721) and 45.2 g. of triethylene glycol di-p-toluene sulfonic acid ester (XVIIa) are heated for 5 hours to 120° C. and further processed according to Example XVIIc. 57.2 g. (62.5 percent of the theory) of a yellowish brown viscous product are obtained.

## COMPOUND XXV

(a) *Ethoxyethyl- $\alpha,\omega$ -Bis-[N,N,N',N'-Tetra-Betyl-N,N'-Di-(Cyanoethoxyethyl)]-Ammonium-Methane Sulfonate*

45.2 g. of dibutyl-cyanoethoxyethyl amine (IIIa) and 26.2 g. of diethylene glycol di-methane sulfonic acid ester (XVIIa) are heated for 4-5 hours to 120° C. and further processed according to Example XVIIc. 50 g. (70 percent of the theory) of a yellowish brown sirupy liquid are obtained.

## COMPOUND XXVI

*Di-(Ethoxy)-Ethyl- $\alpha,\omega$ -Bis-[N,N'-Di-(Cyanoethoxyethyl)]-Morpholinium-p-Toluene Sulfonate*

36.8 g. of  $\beta$ -cyanoethoxyethyl-N-morpholine (described in United States Patent No. 2,326,721) and 45.2 g. of tri-

10  
5

ethylene glycol di-p-toluene sulfonic acid ester (XVIIa) are heated for 5 hours to 120° C. and further processed according to Example XVIIc. 51.5 g. (63 percent of the theory) of a resinous yellowish colored product are obtained.

## 12

## COMPOUND XXVII

(a) *Octaethylene Glycol Di-Methane Sulfonic Acid Ester*

114 g. of methane sulpho-chloride are added in portions at 0° C. to a solution of 185 g. of octa-ethylene-glycol in 200 ml. of dried pyridine, whereby the reaction temperature in the flask should not exceed 5° C. The mixture is stirred for 1½ hours at room temperature and thereafter poured onto 500 g. of ice. The resulting mixture is acidified with hydrogen chloride, saturated with common salt and extracted with methylene chloride. The organic product is separated, clarified with active carbon and bleaching earth and evaporated. The residue represents a yellowish brown viscous product which does not crystallize.

Yield 197 g. (75 percent of the theory).

(b) *Hepta-(Ethoxy)-Ethyl- $\alpha,\omega$ -Bis-[N,N,N',N'-Tetraethyl-N,N'-Di-(Cyanoethoxyethyl)]-Ammonium-Methane Sulfonate*

51 g. of diethyl-cyanoethoxyethyl-amine (IIa) and 52.7 g. of octaethylene glycol di-methane sulfonic acid ester (XXVIIa) are heated with stirring for 3 hours at 120° C. and further processed according to Example XVIIc. 65 g. (75 percent of the theory) of a yellowish brown sirupy liquid are obtained.

## COMPOUND XXVIII

*Hepta-(Ethoxy)-Ethyl- $\alpha,\omega$ -Bis-[N,N'-Dimethyl-N,N'-Tetra-(Cyanoethoxyethyl)]-Ammonium-Methane Sulfonate*

45 g. of di-(cyanoethoxyethyl)-N-methylamine (VIa) and 52.7 g. of octaethylene glycol di-methane sulfonic acid ester (XXVIIa) are heated with stirring for 4 hours to 120° C. and further processed as described in Example XVIIc. 66.5 g. (68 percent of the theory) of a yellowish brown sirupy liquid are obtained.

## COMPOUND XXIX

*Hepta-(Ethoxy)-Ethyl- $\alpha,\omega$ -Bis-[N,N,N',N'-Tetraethyl-N,N'-Di-(Cyanoethoxyethyl)]-Ammonium-Methane Sulfonate*

42.4 g. of diethyl-cyanoethoxypropyl-amine (XXIIa) and 52.7 g. of octaethylene glycol di-methane sulfonic acid ester (XXVIIa) are heated with stirring for 4 hours to 120° C. and further processed according to Example XVIIc. 62 g. (65 percent of the theory) of a yellowish brown sirupy liquid are obtained.

## COMPOUND XXX

*Hepta-(Ethoxy)-Ethyl- $\alpha,\omega$ -Bis-[N,N'-Di-(Cyanoethoxyethyl)]-Morpholinium-Methane Sulfonate*

36.8 g. of cyanoethoxyethyl-N-morpholine (described in United States Patent No. 2,326,721) and 57.2 g. of octaethylene glycol di-methane sulfonic acid ester (XXVIIa) are heated with stirring for 3 hours to 120° C. and further processed as described in Example XVIIc. 64.5 g. (72 percent of the theory) of a resinous yellowish brown product are obtained.

## COMPOUND XXXI

*Hepta-(Ethoxy)-Ethyl- $\alpha,\omega$ -Bis-[N,N'-Diethyl-N,N'-Diphenyl-N,N'-Di-(Cyanoethoxyethyl)]-Ammonium-Methane Sulfonate*

46.4 g. cyanoethoxyethyl-N-phenyl-N-ethyl amine (described in United States Patent No. 2,326,721) and 52.7 g. of octaethylene glycol di-methane sulfonic acid ester (XXVIIa) are heated with stirring for 3 hours to 120°

15  
20  
25  
30  
35  
40  
45  
50  
55  
60  
65  
70  
75

13

C. and further processed according to Example XVIIc. 67.5 g. (68 percent of the theory) of a yellowish brown sirupy liquid are obtained.

The following examples illustrate the effect of the compounds according to the invention. With comparable development times, the accelerator effect is expressed as an increase in sensitivity.

## EXAMPLE 1

A negative gelatino-silver bromide emulsion with a silver coating of 4.5 g. of Ag/m<sup>2</sup> and an iodine content of 66 mmol/mol of Ag and also a content of 920 mg. of 4-hydroxy-6-methyl-1,3,3a,7-tetraazaindene is divided into two portions (A+B). Portion A is cast on a cellulose triacetate film; to portion B are added 0.6 g. of the oleyl polyether derived from 20 mols of ethylene oxide and 1 mol of oleyl alcohol. The resulting emulsion is also cast on a cellulose triacetate film.

The layers are exposed to light behind a stepped wedge with a logarithmic density increase of 0.15 and developed for 5 and 10 minutes, respectively, at 20° C. in a developer of the following composition:

|                                           | G.  |
|-------------------------------------------|-----|
| Anhydrous Na <sub>2</sub> SO <sub>3</sub> | 70  |
| Borax                                     | 7   |
| Hydroquinone                              | 3.5 |
| Metol                                     | 3.5 |
| Sodium citrate                            | 7   |
| KBr                                       | 0.4 |
| Water to make 1000 cc.                    |     |

The layers are thereafter fixed and rinsed.

Under the same conditions, the same layers are developed in developers which contain the substances referred to in the following table in addition to the above composition:

## RESULTS WITH EMULSION A AFTER A DEVELOPMENT TIME OF 5 MINUTES

| Specimen               | Addition, g./l. | Fogging | Sensitivity, <sup>1</sup> degrees | $\gamma^2$ |
|------------------------|-----------------|---------|-----------------------------------|------------|
| Control                |                 | 0.06    |                                   | 0.54       |
| I                      | 1               | 0.06    | +2                                | 0.67       |
| Comparative compound 1 | 0.8             | 0.06    | 0                                 | 0.50       |
| II                     | 1               | 0.06    | +2                                | 0.72       |
| Comparative compound 2 | 0.7             | 0.06    | 0                                 | 0.54       |
| XIII                   | 1               | 0.08    | +2                                | 0.62       |
| Comparative compound 3 | 0.8             | 0.06    | 0                                 | 0.54       |

## RESULTS WITH EMULSION A AFTER 10 MINUTES' DEVELOPMENT

| Specimen               | Addition, g./l. | Fogging | Sensitivity, <sup>1</sup> degrees | $\gamma^2$ |
|------------------------|-----------------|---------|-----------------------------------|------------|
| Control                |                 | 0.07    |                                   | 0.78       |
| XIII                   | 1               | 0.09    | +1.5                              | 0.90       |
| Comparative compound 3 | 0.8             | 0.08    | 0                                 | 0.78       |
| II                     | 1               | 0.07    | +2                                | 0.90       |
| Comparative compound 2 | 0.7             | 0.07    | 0                                 | 0.82       |

## RESULTS WITH EMULSION B AFTER A DEVELOPMENT TIME OF 5 MINUTES

| Specimen               | Addition, g./l. | Fogging | Sensitivity, <sup>1</sup> degrees | $\gamma^2$ |
|------------------------|-----------------|---------|-----------------------------------|------------|
| Control                |                 | 0.06    |                                   | 0.52       |
| II                     | 1               | 0.09    | +1                                | 0.65       |
| Comparative compound 2 | 0.7             | 0.06    | 0                                 | 0.54       |
| XIII                   | 1               | 0.07    | +2                                | 0.65       |
| Comparative compound 3 | 0.8             | 0.08    | -2                                | 0.52       |

## RESULTS WITH EMULSION B AFTER 10 MINUTES' DEVELOPMENT

| Specimen               | Addition, g./l. | Fogging | Sensitivity, <sup>1</sup> degrees | $\gamma^2$ |
|------------------------|-----------------|---------|-----------------------------------|------------|
| Control                |                 | 0.08    |                                   | 0.90       |
| II                     | 1               | 0.08    | +1                                | 0.98       |
| Comparative compound 2 | 0.7             | 0.09    | 0                                 | 0.90       |
| XIII                   | 1               | 0.09    | +2                                | 0.91       |
| Comparative compound 3 | 0.8             | 0.21    | -1                                | 0.83       |

<sup>1</sup> The differences in sensitivity are indicated in degrees DIN; S=0.1 over fogging was selected as measurement point.

<sup>2</sup> The gradation was measured as a straight line between the measurement points S=0.5 and 1.5 over fogging.

<sup>3</sup> Equimolar to XIII.

<sup>4</sup> Equimolar to II.

14

The comparative compounds have the following chemical constitution:

COMPARATIVE COMPOUND 1.—DIMETHYL-PHEN-ETHYL- $\beta$ -HYDROXYETHYL-AMMONIUM CHLORIDE

8.5 g. of N,N-dimethylaminoethanol and 14 g. of  $\omega$ -chlorethyl benzene are heated for 2 hours to 100° C. The reaction product is recrystallized from acetone/alcohol (10:1).

Melting point: 92–93° C. Yield: 16 g.

COMPARATIVE COMPOUND 2.—DIETHYL-BENZYL- $\beta$ -HYDROXYETHYL-AMMONIUM CHLORIDE

15 58.5 g. of N,N-diethylaminoethanol and 63.5 g. of benzyl chloride are heated under reflux for 8 hours in 60 cc. of dry toluene. The oil which is separated out is thereafter heated to boiling point in 100 cc. of acetone. Crystals with the melting point 91 to 92° C.

Yield: 91 g.

COMPARATIVE COMPOUND 3.—1,6-HEXAMETHYLENE-BIS - N,N,N',N' - TETRAMETHYL-N,N'- $\beta$ -DI-HYDROXY-ETHYL-AMMONIUM BROMIDE

16 17.8 g. of N,N-dimethyl-aminoethanol and 24.4 g. of 1,6-dibromohexane are heated for 2 hours to 100° C.

35 The reaction product is recrystallized from alcohol.

Melting point: 179–180° C. Yield: 30 g.

## EXAMPLE 2

An orthochromatically sensitized miniature film strip (Agfa Agepe) exposed behind a stepped wedge is developed for 3 minutes at 20° C. in a developer having the following composition:

|                                           | G.  |
|-------------------------------------------|-----|
| Anhydrous Na <sub>2</sub> SO <sub>3</sub> | 50  |
| Hydroquinone                              | 6.5 |
| Anhydrous Na <sub>2</sub> CO <sub>3</sub> | 40  |
| NaBr                                      | 5   |
| 1-phenyl-3-pyrazolidone                   | 0.3 |
| Water to make 1000 cc.                    |     |

50 The strip is thereafter fixed and rinsed.

Under the same conditions, the same film is developed in a developer which additionally contains 0.25 g. of the Compound VI per litre.

| Specimen | Addition, g./l. | Fogging | Sensitivity, <sup>1</sup> degrees | $\gamma^2$ |
|----------|-----------------|---------|-----------------------------------|------------|
| Control  | 0.25            | 0.05    | +2                                | 2.9        |
| VI       | 0.3             |         |                                   | 3.5        |

<sup>1</sup> Sensitivity at S=1.

<sup>2</sup> Gradation between the measurement points S=0.7 and 2.0.

## EXAMPLE 3

A panchromatically sensitized miniature film strip (Agfa Isopan IFF) exposed behind a stepped wedge is developed for 3 minutes at 20° C. in a developer having the following composition:

|                                           | G.  |
|-------------------------------------------|-----|
| Anhydrous Na <sub>2</sub> SO <sub>3</sub> | 50  |
| Hydroquinone                              | 6.5 |
| Anhydrous Na <sub>2</sub> CO <sub>3</sub> | 40  |
| NaBr                                      | 5   |
| 1-phenyl-3-pyrazolidone                   | 0.3 |
| Water to make 1000 cc.                    |     |

75 The strip is then fixed and rinsed.

## 15

Under the same conditions, the same film is developed in a developer which also contains 0.8 of the Compound IV per litre.

| Specimen | Addition, g./l. | Fogging | Sensitivity, <sup>1</sup> degrees | $\gamma^2$ |
|----------|-----------------|---------|-----------------------------------|------------|
| Control  |                 | 0.27    |                                   | 1.2        |
| IV       | 0.8             | 0.27    | +2                                | 2.0        |

<sup>1,2</sup> As in Example 2.

## EXAMPLE 4

A highly sensitive film (Agfa X-ray dental film) coated on both sides and disposed beneath an aluminium step, is exposed with X-ray radiation and developed for 3 minutes at 20° C. in the developer referred to in Example 2. Under the same conditions, the same film is developed in a developer which also contains 0.25 g. of the substance III per litre.

| Specimen | Addition, g./l. | Fogging | Sensitivity, <sup>1</sup> degrees | $\gamma^2$ |
|----------|-----------------|---------|-----------------------------------|------------|
| Control  |                 | 0.11    |                                   | 1.1        |
| III      | 0.25            | 0.13    | +3                                | 1.1        |

<sup>1,2</sup> As in Example 2.

## EXAMPLE 5

An orthochromatically sensitized miniature film strip (Agfa Agepe) exposed behind a stepped wedge is developed for 3 minutes at 20° C. in a developer having the following composition:

|                                                                     |     |
|---------------------------------------------------------------------|-----|
| Anhydrous Na <sub>2</sub> SO <sub>3</sub>                           | 50  |
| Hydroquinone                                                        | 6.5 |
| Anhydrous Na <sub>2</sub> CO <sub>3</sub>                           | 40  |
| NaBr                                                                | 5   |
| 1 - p-aminophenyl - 3-amino- $\Delta^2$ -pyrazoline-dihydrochloride | 0.2 |
| Water to make 1000 cc.                                              |     |

The strip is then fixed and rinsed.

Under the same conditions, the same film is developed in a developer which also contains 0.8 g. of the substance IV per litre.

| Specimen | Addition, g./l. | Fogging | Sensitivity, <sup>1</sup> degrees | $\gamma^2$ |
|----------|-----------------|---------|-----------------------------------|------------|
| Control  |                 | 0.08    |                                   | 3.0        |
| IV       | 0.8             | 0.06    | +2                                | 3.0        |

<sup>1,2</sup> As in Example 2.

## EXAMPLE 6

A highly sensitive film (Agfa X-ray dental film) coated on both sides and disposed beneath an aluminium step is exposed to X-ray radiation and fixed and developed for 7 minutes at 20° C. with vigorous movement in a combined fixer and developer of the following composition:

|                                                                  |        |
|------------------------------------------------------------------|--------|
| Anhydrous Na <sub>2</sub> SO <sub>3</sub>                        | g. 30  |
| Hydroquinone                                                     | g. 14  |
| 1-phenyl-3-pyrazolidone                                          | g. 0.5 |
| Na <sub>3</sub> PO <sub>4</sub> .12H <sub>2</sub> O              | g. 60  |
| Na <sub>2</sub> S <sub>2</sub> O <sub>3</sub> .5H <sub>2</sub> O | g. 50  |
| NaBr                                                             | g. 10  |
| Normal sodium hydroxide solution                                 | cc. 50 |
| Water to make 1000 cc.                                           |        |

In the same way, the same film is developed in the

## 16

forementioned combined fixer and developer, which also contains the substances I, VII or IX.

| Specimen | Addition, g./l. | Fogging | Sensitivity, <sup>1</sup> degrees | $\gamma^2$ |
|----------|-----------------|---------|-----------------------------------|------------|
| Control  | 0.1             | 0.25    |                                   | 0.76       |
| I        | 0.1             | 0.29    | +5                                | 0.90       |
| VII      | 0.1             | 0.25    | +3                                | 0.85       |
| IX       | 0.1             | 0.24    | +2                                | 0.90       |
| IX       | 0.25            | 0.28    | +5                                | 0.90       |

<sup>1,2</sup> As in Example 2.

## EXAMPLE 7

An orthochromatically sensitized miniature film strip (Agfa Agepe) exposed behind a stepped wedge is fixed and developed with brisk moving in a combined fixer and developer of the following composition for 7 minutes at 20° C.:

|                                                                  |        |
|------------------------------------------------------------------|--------|
| Anhydrous Na <sub>2</sub> SO <sub>3</sub>                        | g. 30  |
| Hydroquinone                                                     | g. 14  |
| 1-phenyl-3-pyrazolidone                                          | g. 0.5 |
| Na <sub>3</sub> PO <sub>4</sub> .12H <sub>2</sub> O              | g. 60  |
| Na <sub>2</sub> S <sub>2</sub> O <sub>3</sub> .5H <sub>2</sub> O | g. 60  |
| NaBr                                                             | g. 10  |
| Normal sodium hydroxide solution                                 | cc. 50 |
| Water to make 1000 cc.                                           |        |

Under the same conditions, the same film is developed in a combined fixer and developer which also contains 0.5 g. of the substance II per litre.

| Specimen | Addition, g./l. | Fogging | Sensitivity, <sup>1</sup> degrees | $\gamma^2$ |
|----------|-----------------|---------|-----------------------------------|------------|
| Control  |                 | 0.05    |                                   | 1.8        |
| II       | 0.5             | 0.10    | +3                                | 1.8        |

<sup>1,2</sup> As in Example 2.

## EXAMPLE 8

A panchromatically sensitized miniature film strip (Agfa Isopan IFF) exposed behind a stepped wedge is fixed and developed for 7 minutes at 20° C. with vigorous movement in a combined fixer and developer of the following composition:

|                                                                  |        |
|------------------------------------------------------------------|--------|
| Anhydrous Na <sub>2</sub> SO <sub>3</sub>                        | g. 30  |
| Hydroquinone                                                     | g. 14  |
| 1-phenyl-3-pyrazolidone                                          | g. 0.5 |
| Na <sub>3</sub> PO <sub>4</sub> .12H <sub>2</sub> O              | g. 60  |
| Na <sub>2</sub> S <sub>2</sub> O <sub>3</sub> .5H <sub>2</sub> O | g. 50  |
| NaBr                                                             | g. 10  |
| Normal sodium hydroxide solution                                 | cc. 50 |
| Water to make 1000 cc.                                           |        |

Under the same conditions, the same film is developed in a combined fixer and developer which also contains 0.25 or 0.5 g. of the substance II per litre.

| Specimen | Addition, g./l. | Fogging | Sensitivity, <sup>1</sup> degrees | $\gamma^2$ |
|----------|-----------------|---------|-----------------------------------|------------|
| Control  |                 | 0.25    |                                   | 1.2        |
| II       | 0.25            | 0.26    | +3.5                              | 1.3        |
| II       | 0.5             | 0.26    | +3                                | 1.3        |

<sup>1,2</sup> As in Example 2.

## EXAMPLE 9

A highly sensitive film (AGFA X-ray dental film) coated on both sides and disposed beneath an aluminium step is exposed with X-ray radiation and fixed and developed for 7 minutes at 20° C. with vigorous movement

## 17

in a combined fixer and developer having the following composition:

|                                                                         |        |
|-------------------------------------------------------------------------|--------|
| Anhydrous $\text{Na}_2\text{SO}_3$ -----                                | g. 30  |
| Hydroquinone -----                                                      | g. 14  |
| 1-(p-aminophenyl)-3-amino- $\Delta^2$ -pyrazoline-dihydrochloride ----- | g. 0.3 |
| $\text{Na}_3\text{PO}_4 \cdot 12\text{H}_2\text{O}$ -----               | g. 60  |
| $\text{Na}_2\text{S}_2\text{O}_3 \cdot 5\text{H}_2\text{O}$ -----       | g. 50  |
| NaBr -----                                                              | g. 10  |
| Normal sodium hydroxide solution-----                                   | cc. 50 |
| Water to make 1000 cc.                                                  | 10     |

Under the same conditions, the same film is developed in a combined fixer and developer which also contains the substances II, III, VII, or VIII.

| Specimen     | Addition, g./l. | Fogging | Sensitivity, <sup>1</sup> degrees | $\gamma^2$ |
|--------------|-----------------|---------|-----------------------------------|------------|
| Control----- |                 | 0.26    |                                   | 0.9        |
| II-----      | 0.2             | 0.24    | +2                                | 0.9        |
| III-----     | 0.2             | 0.24    | +3.5                              | 0.9        |
| VII-----     | 0.2             | 0.21    | +2                                | 0.9        |
| VIII-----    | 0.05            | 0.24    | +3.5                              | 0.9        |

<sup>1,2</sup> As in Example 2.

## EXAMPLE 10

A color positive film strip (Agfa Color Positive Cinema Type S) exposed behind a stepped wedge is developed for 8 minutes at 20° C. in a color developer of the following composition:

|                                           | G.   |
|-------------------------------------------|------|
| Diethyl-p-phenylene diamine sulphate----- | 2.75 |
| Hydroxylamine sulphate-----               | 1.2  |
| Anhydrous sodium sulphite-----            | 2.0  |
| Sodium hexametaphosphate-----             | 2.0  |
| Anhydrous potassium carbonate-----        | 75   |
| Potassium bromide-----                    | 2.0  |
| Water to make 1000 cc.                    |      |

After the usual further processing by means of a bleaching bath and fixing bath, a measurable color wedge is obtained.

Under the same conditions, the same film is developed in the above developer, which also contains the substances I or II. The accelerating effect is apparent from the following table:

| Specimen     | Addition, g./l. | Fogging                    | Sensitivity, <sup>1</sup> degrees | $\gamma^2$        |
|--------------|-----------------|----------------------------|-----------------------------------|-------------------|
| Control----- |                 | y 0.12<br>m 0.07<br>c 0.08 | 2.2<br>2.2<br>2.8                 |                   |
| I-----       | 1               | y 0.16<br>m 0.09<br>c 0.11 | +2<br>+3<br>+2                    | 2.6<br>2.8<br>3.3 |
| II-----      | 0.5             | y 0.14<br>m 0.08<br>c 0.10 | +1.5<br>+1.5<br>+1                | 3.0<br>3.0<br>3.5 |

<sup>1</sup> Sensitivity measured at S=0.1 over fogging.

<sup>2</sup> Gradation measured between the measurement S=0.7 and 2.0 over fogging.

NOTE.—y=yellow, m=magenta, c=cyan.

## EXAMPLE 11

A silver bromide paper (Agfa Brovira Normal 1) exposed behind a stepped wedge with a logarithmic density increase of 0.1 is developed for 60 seconds at 20° C. in a developer of the following composition and fixed and rinsed in the usual manner.

|                                 | G. |
|---------------------------------|----|
| Anhydrous sodium sulphite-----  | 13 |
| Hydroquinone -----              | 3  |
| Monomethyl-p-amino-phenol ----- | 1  |
| Anhydrous soda-----             | 26 |
| KBr -----                       | 1  |
| Water to make 1000 cc.          | 75 |

## 18

Under the same conditions, the same paper strip is developed in a developer which also contains 0.2 g. of the Compound XIII per litre. The strip has the sensitivity and gradation of the comparison strip after 50 seconds; at 60 sec. it shows a sensitivity which is higher by one step.

## EXAMPLE 12

A panchromatically sensitized gelatino-silver bromide negative emulsion, containing 0.35 mol of silver halide per litre of casting solution and having a sensitivity of 21° DIN was divided into two portions.

Portion A was cast as a comparison test with a casting thickness of 11 $\mu$  on a cellulose triacetate support, provided with a subbing layer.

Portion B had added thereto 1.5 g. of the Compound II per litre of casting solution and was cast with the same layer thickness.

Both film samples, after exposure behind a grey stepped wedge, were developed under comparable conditions as regards temperature and movement in a developer having the following composition:

|                                             | G.  |
|---------------------------------------------|-----|
| Ortho-hydroxyethylaminophenolsulphate ----- | 7.5 |
| Anhydrous sodium sulphite-----              | 100 |
| Anhydrous soda-----                         | 10  |
| KBr -----                                   | 0.4 |
| Water to make 1000 cc.                      |     |

## RESULTS OF THE DEVELOPMENT AFTER 12 MINUTES' DEVELOPMENT TIME AT 20° C.

|              |                             | Sensitivity, degrees | Gradation  | Fogging      |
|--------------|-----------------------------|----------------------|------------|--------------|
| Control----- | Portion A<br>Portion B----- | +1                   | 0.5<br>0.8 | 0.10<br>0.11 |

## RESULTS OF THE DEVELOPMENT AFTER A DEVELOPMENT TIME OF 24 MINUTES AT 20° C.

|              | Portion A<br>Portion B----- | +1.5 | 0.85<br>0.25 | 0.13 |
|--------------|-----------------------------|------|--------------|------|
| Control----- |                             |      |              |      |

## EXAMPLE 13

A panchromatically sensitized photographic film (Agfa Isopan IFF) is exposed through a test wedge, developed for 10 minutes at 20° C., fixed and washed. The developer has the following composition:

|                                           | G.  |
|-------------------------------------------|-----|
| $\text{Na}_2\text{SO}_3$ anhydrous -----  | 70  |
| Borax -----                               | 7   |
| Hydroquinone -----                        | 3.5 |
| Metol (p-methylaminophenol sulfate) ----- | 3.5 |
| Sodium citrate -----                      | 7   |
| KBr -----                                 | 0.4 |
| Water to make 1000 cc.                    |     |

Samples of the same photographic material are processed under the same conditions with the only exception that the developer additionally contains a certain amount of the Compounds XVII-XX. The improving of the sensitivity is indicated in degrees DIN; as measurement point is selected S=0.2 over fogging. The gradation is measured as a straight line between the measurement point S=0.5 and 1.5 over fogging.

| Sample       | Addition, g./l. | Improvement of Sensitivity, degrees | $\gamma$ | Fogging |
|--------------|-----------------|-------------------------------------|----------|---------|
| Control----- |                 |                                     |          |         |
| XVII-----    | 1               | +2                                  | 0.9      | 0.05    |
| XVIII-----   | 1               | +1.5                                | 1.1      | 0.06    |
| XIX-----     | 1               | +2                                  | 1.1      | 0.06    |
| XX-----      | 1               | +2                                  | 1.1      | 0.06    |

**19**  
**EXAMPLE 14**

A panchromatically sensitized photographic film (Agfa Isopan ISS) is processed according to Example 13. Comparative tests with the same photographic material using the developer composition described above with an additional content of Compounds XVII-XX show the following results:

| Sample  | Addition, g./l. | Improvement of Sensitivity, degrees | $\gamma$ | Fogging |
|---------|-----------------|-------------------------------------|----------|---------|
| Control |                 |                                     | 0.7      | 0.09    |
| XVII    | 1               | +2                                  | 0.8      | 0.12    |
| XVIII   | 1               | +2                                  | 0.8      | 0.12    |
| XIX     | 1               | +2                                  | 0.8      | 0.12    |
| XX      | 1               | +2                                  | 0.8      | 0.12    |

**EXAMPLE 15**

A silver bromide gelatine negative emulsion (66 millimols AgI/Mol AgBr) which is not additionally sensitized is cast on a cellulose triacetate support. The resulting layer has a silver content of 4.5 g. Ag/m<sup>2</sup>. The material is exposed through a test wedge and developed for 1 minute at 20° C. in a developer having the following composition:

|                                           | G.  |
|-------------------------------------------|-----|
| Hydroquinone                              | 3   |
| Na <sub>2</sub> SO <sub>3</sub> anhydrous | 20  |
| Phenidone (1-phenyl-3-pyrazolidone)       | 0.4 |
| Na <sub>2</sub> CO <sub>3</sub> anhydrous | 20  |
| KBr                                       | 1   |
| Benzotriazole                             | 0.1 |
| Water to make 1000 cc.                    |     |

Comparative tests with developers which additionally contain Compounds XVII-XX show the following results:

| Sample  | Addition, g./l. | Improvement of Sensitivity, degrees | $\gamma$ | Fogging |
|---------|-----------------|-------------------------------------|----------|---------|
| Control |                 |                                     | 0.63     | 0.04    |
| XVII    | 1               | +1.5                                | 0.65     | 0.05    |
| XVIII   | 1               | +2.5                                | 0.67     | 0.05    |
| XIX     | 1               | +2                                  | 0.65     | 0.05    |
| XX      | 1               | +2                                  | 0.65     | 0.05    |

**EXAMPLE 16**

A silver bromide gelatine emulsion having an iodine content of 25 mmol/mol Ag is divided into two portions (A and B). Portion A is cast on a suitable support without any further addition; to portion B is added before casting 0.5 g. of the Compounds XX/kg. of emulsion. Strips of said two film materials were exposed through a test wedge, developed, fixed, washed and dried. The developer has the following composition:

|                                           | G.  |
|-------------------------------------------|-----|
| Na <sub>2</sub> SO <sub>3</sub> anhydrous | 70  |
| Borax                                     | 7   |
| Hydroquinone                              | 3.5 |
| Metol (p-methylaminophenol sulfate)       | 3.5 |
| Sodium citrate                            | 7   |
| KBr                                       | 0.4 |
| Water to make 1000 cc.                    |     |

After the usual processing (fixing, washing, drying) the following results are obtained:

| Sample | Addition, g./l. | Improvement of Sensitivity, degrees | $\gamma$ | Fogging |
|--------|-----------------|-------------------------------------|----------|---------|
| A      | 0.5             | +2                                  | 0.8      | 0.03    |
| B      | 0.5             | +2                                  | 0.9      | 0.05    |

**20**  
**EXAMPLE 17**

Similar results as in Example 16 are obtained if the following developer composition is used:

|                                                                      | G.  |
|----------------------------------------------------------------------|-----|
| 5 Na <sub>2</sub> SO <sub>3</sub> anhydrous                          | 50  |
| Hydroquinone                                                         | 6.5 |
| Na <sub>2</sub> CO <sub>3</sub> anhydrous                            | 40  |
| 1 (p - amino-phenyl)-3-amino- $\Delta^2$ -pyrazoline-dihydrochloride | 0.2 |
| 10 Water to make 1000 cc.                                            |     |

The following result was obtained:

| Sample | Addition, g./kg., Emulsion | Improvement of Sensitivity, degrees | $\gamma$ | Fogging |
|--------|----------------------------|-------------------------------------|----------|---------|
| A      | 0.5                        | +2                                  | 1.2      | 0.03    |
| B      | 0.5                        | +2                                  | 1.8      | 0.06    |

**EXAMPLE 18**

The following example demonstrates the superiority of the compounds whose use is specified in the present invention in comparison with corresponding compounds which contain no cyanoethoxy radical. The tests were performed with the film material described in Example 15. The negative film is developed for 5 minutes at 20° C. with the developer described in Example 13. After the usual fixing and washing, the following results were obtained:

| Sample               | Addition, g./l. | Improvement of Sensitivity, degrees | $\gamma$ | Fogging |
|----------------------|-----------------|-------------------------------------|----------|---------|
| Control              |                 |                                     | 0.6      | 0.05    |
| Comparative Compound | 0.37            | +1                                  | 0.70     | 0.06    |
| Compound XXVII       | 0.42            | +2                                  | 0.86     | 0.06    |
| Compound XXVIII      | 0.50            | +2                                  | 0.85     | 0.07    |

The comparative compound hepta-(ethoxy)-ethyl- $\alpha$ , $\omega$ -bistriethylammonium-methane sulfonate:



is used.

The compound is prepared according to the following instructions: 52.7 g. of octaethylene glycol di-methane sulfonic acid ester (XXVIIb) and 40.4 g. of triethylamine are refluxed for 5 hours in 50 cc. of acetone. After evaporating the solvent and the excess of triethylamine, the reaction mixture is extracted for three times with benzene, dissolved in methanol and treated with active carbon, bleaching earth and again with active carbon. After evaporating in vacuo 59 g. (81 percent of the theory) of a yellowish brown-colored highly viscous oil are obtained. A 20 percent aqueous solution is used for the photographic test.

**EXAMPLE 19**

A strip of a color-positive-film (Agfa-color-positive cinefilm type S) is exposed through a test wedge and developed for 8 minutes at 20° C. with a color-forming developer having the following composition:

|                                       | G.   |
|---------------------------------------|------|
| Diethyl-p-phenylene diamine-sulfonate | 2.75 |
| Hydroxylamine sulfate                 | 1.2  |
| Sodium sulfite anhydrous              | 2.0  |
| Sodium hexametaphosphate              | 2.0  |
| Potassium carbonate anhydrous         | 75   |
| Water to make 1000 cc.                |      |

A strip of the same film material is processed under the same conditions with the only exception that the de-

veloper composition described above contains additionally a certain amount of the Compound XXVIII. The following results are obtained:

| Sample               | Addition, g./l. | Improvement of Sensitivity <sup>1</sup>                     | $\gamma^2$        | Fogging              |
|----------------------|-----------------|-------------------------------------------------------------|-------------------|----------------------|
| Control.....         |                 | y -<br>m -<br>c -                                           | 2.4<br>2.4<br>2.8 | 0.12<br>0.08<br>0.07 |
| Compound XXVIII..... | 0.5             | y + <sup>20</sup><br>m + <sup>20</sup><br>c + <sup>20</sup> | 2.7<br>2.7<br>3.1 | 0.17<br>0.10<br>0.09 |

<sup>1</sup> Sensitivity measured at  $S=0.2$  over fogging.

<sup>2</sup> Gradation measured between the measurement  $S=0.7$  and 2.0 over fogging.

#### EXAMPLE 20

A silver bromide gelatine emulsion having an iodide content of 60 mmol/mol Ag which contains a cyan coupler of the naphthol series for example 2-(N-methyl-N-n-octadecyl)amino-5-sulfo-1'-hydroxy-2'-naphthalide is divided in three portions.

Portion A is cast on a suitable support with a thickness of the layer of  $5\mu$ . To portion B is added 0.5 g. of the Compound XX/kg. of emulsion. To portion C is added 0.5 g. of the Compound XXVIII/kg. of emulsion.

The resulting layers of B and C have also a thickness of  $5\mu$ . The three samples are exposed through a test wedge and developed under the same conditions for 8 minutes in the color-forming developer described in Example 19. After the usual further processing by means of a bleaching and fixing bath the following results are obtained:

| Sample | Addition, g./kg., Emulsion | Improvement of Sensitivity, <sup>1</sup> degrees | $\gamma^2$ | Fogging |
|--------|----------------------------|--------------------------------------------------|------------|---------|
| A..... |                            |                                                  | 0.7        | 0.10    |
| B..... | 0.5                        | +2                                               | 0.8        | 0.10    |
| C..... | 0.5                        | +3                                               | 1.1        | 0.11    |

<sup>1</sup> As in Example 19.

hydroquinone, p-methylamino phenol, 1-phenylpyrazolide-3 and derivatives thereof, compounds of the 4-aminopyrazolone series, 1-aminophenyl-3-amino-pyrazoline and derivatives thereof or color-forming developers of the p-phenylene diamine type. According to one embodiment of the invention, the development can be accomplished in the presence of silver halide solvents such as water-soluble alkali-metal, alkaline-earth-metal or ammonium thiosulfates, in particular sodium, potassium or ammonium thiosulfate. The compounds according to the invention can be added to the developer composition in an amount of 0.01-10 g. per litre or to a silver halide emulsion in an amount of 0.1-10 g. per kg. of emulsion.

What we claim is:

1. In a process for developing an exposed photographic material containing at least one silver halide emulsion layer, the improvement which consists in developing the exposed photographic material in contact with a compound having the formula



25 in which  $R_1$  and  $R_2$  are each a radical of the group consisting of alkyl, phenylalkyl, phenyl, cyanoethyl, and cyanoethoxyethyl and together are the atoms required to complete a heterocyclic radical of the group consisting of morpholino and piperidino;  $R_3$  is a member of the group 30 consisting of alkyl, phenylalkyl, phenyl, cyanoethoxyethyl and radicals having the following formulae



and



wherein  $m$  is an integer from 2 to 5,  $n$  is an integer from 2 to 6 and  $p$  is an integer from 1 to 100; and  $X$  is an anion.

2. A process as defined in claim 1 in which the exposed photographic material is developed in contact with a compound having the following formula



wherein  $R_1$  and  $R_2$  are each a radical of the group consisting of alkyl, phenylalkyl, phenyl, cyanoethyl, and cyanoethoxyethyl and together are the atoms required to complete a heterocyclic ring, wherein  $m$  is an integer from 2 to 5 and  $p$  is an integer from 1 to 7, and  $X$  is an anion.

3. A process as defined in claim 1 in which the exposed photographic material is developed in contact with a silver halide solvent.

4. A process as defined in claim 1 in which the exposed photographic material is developed in contact with a poly-alkylene oxide.

5. A light-sensitive photographic material having at least one light-sensitive silver halide emulsion layer and containing between 0.1 and 10 grams per kilogram of the said emulsion of a compound of the following formula



75 in which  $R_1$  and  $R_2$  are each a radical of the group consisting of alkyl, phenylalkyl, phenyl, cyanoethyl, and cyanoethoxyethyl and together are the atoms required to complete a heterocyclic radical of the group consisting of

<sup>1</sup> As in Example 19.

Having thus described our invention, we now state that we believe our invention to be capable of numerous variations. For example, the compounds according to the invention can be used in combination with any developer compound or composition known per se; e.g.,

23

morpholino and piperidino; R<sub>3</sub> is a member of the group consisting of alkyl, phenylalkyl, phenyl, cyanoethoxyethyl and radicals having the following formulae



and



wherein m is an integer from 2 to 5, n is an integer from 2 to 6 and p is an integer from 1 to 100; and X is an anion.

6. An aqueous developer composition containing a compound of the following formula



in which R<sub>1</sub> and R<sub>2</sub> are each a radical of the group consisting of alkyl, phenylalkyl, phenyl, cyanoethyl, and cy-

5

24

anoethoxyethyl and together are the atoms required to complete a heterocyclic radical of the group consisting of morpholino and piperidino; R<sub>3</sub> is a member of the group consisting of alkyl, phenylalkyl, phenyl, cyanoethoxyethyl and radicals having the following formulae



10 and



wherein m is an integer from 2 to 5, n is an integer from 2 to 6 and p is an integer from 1 to 100; and X is an anion.

## References Cited in the file of this patent

## UNITED STATES PATENTS

- |    |           |                      |                |
|----|-----------|----------------------|----------------|
| 20 | 2,482,546 | Kaszuba -----        | Sept. 20, 1949 |
|    | 2,944,902 | Carroll et al. ----- | July 12, 1960  |
|    | 3,047,389 | Dickinson -----      | July 13, 1962  |